

# United States Patent Office

3,522,052  
Patented July 28, 1970

1

3,522,052  
PHOTOGRAPHIC SUPERSENSITIZED SILVER  
HALIDE EMULSIONS

Keisuke Shiba and Masanao Hinata, Kanagawa, Japan,  
assignors to Fuji Shashin Film Kabushiki Kaisha, Kanagawa, Japan

No Drawing. Filed Nov. 7, 1966, Ser. No. 592,292  
Claims priority, application Japan, Nov. 6, 1965,  
40/68,012

U.S. Cl. 96—104

Int. Cl. G03c 1/28

4 Claims

## ABSTRACT OF THE DISCLOSURE

A super-sensitized photographic silver halide emulsion containing at least one optical sensitizer represented by general Formula I below and at least one optical sensitizer represented by general Formula II below.



The individual moieties above are defined in the claims.

The present invention relates to a photographic silver halide sensitized by the combination of two types of optical sensitizers and more particularly to an optical sensitized red-sensitive emulsion of light-sensitive color elements.

A multiple layer, light-sensitive color element, of the subtractive color processing type, usually comprises at least a blue-sensitive emulsion layer, a green-sensitive emulsion layer, and a red-sensitive emulsion layer. For obtaining good color reproduction with such a light-sensitive color element, the sensitizing ranges of the three layers must be sufficiently separated. Also, for this purpose, a red-sensitive emulsion layer having low green sensitivity, but high red sensitivity, is required. Further, the optical sensitizer used in the red-sensitive emulsion layer must not be diffused from said layer into other layers to give red sensitivity to the diffused layers. To obtain a high-sensitive color element, such an optical sensitizing method is required that gives high optical sensitization and is not accompanied by a reduction in optical sensitization owing to the presence of a coupler in the optical-sensitized light-sensitive emulsion layer and by a reduction in sensitivity with the lapse of time. The objects of this invention are to fulfill the above requirements.

The inventors have found that by using simultaneously the two types of the optical sensitizers shown below, the above objects of this invention can be successfully accomplished and in this manner an excellent red sensitivity can be obtained by a super-sensitization effect.

The photographic light-sensitive silver halide emulsion of the present invention is optically-sensitized by at least one optical sensitizer represented by the following general formula, Formula I, and at least one optical sensitizer represented by the following general formula, Formula II,

2

Formula I



and

Formula II



wherein R<sub>1</sub>, R<sub>2</sub>, R<sub>3</sub> and R<sub>4</sub> each represents a lower alkyl group, a substituted alkyl group, an allyl group, an aralkyl group or a substituted aralkyl group, but, at least one of said groups R<sub>1</sub>, R<sub>2</sub>, R<sub>3</sub> and R<sub>4</sub> is a carboxyalkyl group or the derivative thereof, or a sulfoalkyl group or the derivative thereof; V represents a halogen atom, X represents an anion, or the derivative thereof; V represents a halogen atom, and n is 1 or 2.

Illustrative of suitable substituted alkyl groups,  $\beta$ -hydroxyethyl,  $\beta$ -acetoxyethyl,  $\gamma$ -acetoxypropyl, ethylsulfate, propylsulfate, and the like, or carboxyalkyl, derivatives of a carboxyalkyl, sulfoalkyl, and derivatives of sulfoalkyl that have been defined above as being at least one of said groups R<sub>1</sub>, R<sub>2</sub>, R<sub>3</sub>, and R<sub>4</sub>. As the carboxyalkyl group or derivative thereof, suitable groups are, for example, carboxymethyl,  $\beta$ -carboxyethyl,  $\gamma$ -carboxypropyl, 2-(2-carboxyethoxy)-ethyl and the like. As the sulfoalkyl group or derivative thereof, suitable groups are, for example,  $\beta$ -sulfonybutyl,  $\gamma$ -sulfonypropyl,  $\delta$ -sulfomethyl, 2-hydroxy-1-sulfonypropyl, 3-methoxy-2-(3-sulfonypropoxy)propyl, 2[2(3-sulfonypropoxy)ethoxy]ethyl and 2-hydroxy-3-(3-sulfonypropoxy)propyl.

The optical sensitizer shown by general Formula I has been known as a panchromatic optical sensitizer. In particular, if a sulfoalkyl group or a carboxyalkyl group is introduced into at least one of group R<sub>1</sub> and group R<sub>2</sub>, the reduction in optical sensitization caused by the presence of a coupler can be reduced. However, in the case of using the optical sensitizer there are certain drawbacks such that the extent of the improvement of the optical sensitivity by improving the reduction of optical sensitization is too little to accomplish the objects of the present invention, and the diffusion of the optical sensitizer into other layers is promoted by the reduction in the adsorption power for silver halides together with an increase in the hydrophilic property.

The optical sensitizer represented by general Formula II, that is,  $\beta$ -naphthothiacyanine has a longer color sensitive wave length range than that of the optical sensitizer represented by general Formula I, which is not desirable for color reproduction.

The inventors have found, however, that by using optical sensitizer I together with optical sensitizer II, they exhibit a very remarkable color sensitizing function and, hence, an extremely high color sensitization can be obtained. That is, by incorporating in a silver halide light-sensitive emulsion both optical sensitizer I and optical sensitizer II, there is exhibited a marked increase in red sensitization and a maximum optical sensitizing wave length in an intermediate range between those obtained in the cases of using the optical sensitizers individually. This makes it possible to change desirably the sensitivity distribution of the maximum optical sensitizing wave length range by changing the ratio of both color sensitizers.

The ratio of the proportion of optical sensitizer I to the proportion of optical sensitizer II in this invention has no specific limitation and may be suitably varied in a range of 9:1 to 1:9 according to the purpose. Further, the use of two such optical sensitizers that have not a sulfoalkyl group, a derivative of the sulfoalkyl group, a carboxyalkyl group or a derivative of the carboxyalkyl group in any of groups R<sub>1</sub>, R<sub>2</sub>, R<sub>3</sub>, and R<sub>4</sub>, said optical sensitizers



not being included among the optical sensitizers of the invention, results in a weak super-optical sensitization. The sensitization is too weak and the green sensitivity is considerably increased with the increase in red sensitivity by the addition of these sensitizers. This makes the use of such optical sensitizers undesirable for the objects of this invention (Cf. Example 1). The super-optical sensitization by the use of optical sensitizer I and optical sensitizer II, according to the present invention, has great merit in that the green sensitivity is not increased as compared with the remarkable increase in red sensitivity. Furthermore, it is also an important feature of the present invention that the diffusion of optical sensitizers, from the emulsion layer containing them into other emulsion layers, is prevented, as compared with the case of incorporating in the layer optical sensitizer I or optical sensitizer II. Moreover, the reduction in red sensitivity which is liable to occur during preservation in a sensitizer-containing emulsion layer of a light-sensitive color element is decreased.

The super-optical sensitization achieved by the present invention is scarcely disturbed by coexistence in a silver halide emulsion with a compound having an acid group, such as, a sulfonic acid group or a carboxyl group, for example, a surface active agent, a high molecular sensitizer or a flocculating agent. Furthermore, by the addition of pseudocyanine, oxacarbocyanine, or imidacarbocyanine in the silver halide emulsion containing the two optical sensitizers, according to the present invention, a highly sensitive super-panchromatic optical sensitivity can be obtained.

Examples of typical optical sensitizers used in this invention are illustrated below, although the optical sensitizers of this invention are not limited to them:



The present invention will now be further explained in detail and in practice by referring to the following examples:

#### EXAMPLE 1

Into 100 g. of a gelatino bromo-iodide emulsion (AgI 6.0 mol percent), which had been prepared by a conventional method, there was added a  $\frac{1}{1000}$  mol methanol solution of optical sensitizer I-A or optical sensitizer II-A, or there were added a  $\frac{1}{1000}$  mol methanol solution of optical sensitizer I-A and a  $\frac{1}{1000}$  mol methanol solution of optical sensitizer II-A in the amount or amounts shown below in Table 1. Thereafter, the system was stirred for 60 minutes at 40° C. to stabilize the optical sensitization action. Then, after adding a hardening agent, the emulsion was immediately applied to a film support and dried to provide a red-sensitive color element of the type to be developed in a developer container coupler.

The resulting film was cut into strips. The strips were subjected to red exposure through Fuji Filter No. 75 and then to green exposure through Fuji Filter No. 17 by means of a sensitometer at a color temperature of 4800° K., and thereafter were developed in a primary black and white developer having the following composition for color development.

#### Black and white developer:

Metol—4 g.  
Sodium sulfite—50 g.  
Hydroquinone—5 g.



The color film was subjected to a sensitometry as in Example 1 to obtain the red sensitivities and green sensitivities. The results are shown in Table 4.

TABLE 4

| No.    | Amount of 1/1,000 mol methanol soln. of I-B (ml.) | Amount of 1/1,000 mol methanol soln. of II-B (ml.) | Relative green sensitivity | Relative red sensitivity | $\mu$ |
|--------|---------------------------------------------------|----------------------------------------------------|----------------------------|--------------------------|-------|
| 1----- | 2                                                 | 0                                                  | 22.5                       | 100                      | 658   |
| 2----- | 4                                                 | 0                                                  | 32.5                       | 125                      | 658   |
| 3----- | 0                                                 | 2                                                  | 22.0                       | 150                      | 682   |
| 4----- | 0                                                 | 4                                                  | 24.5                       | 180                      | 684   |
| 5----- | 2                                                 | 2                                                  | 53                         | 225                      | 676   |

<sup>1</sup>  $\mu$  = Maximum sensitization wave length.

## EXAMPLE 4

Into 100 g. of a bromo-iodide emulsion (AgI 7.0 mol percent), prepared by a conventional method, there was dissolved a  $\frac{1}{1000}$  mol methanol solution of optical sensitizer I-D or II-C, or there were dissolved a  $\frac{1}{1000}$  mol methanol solution of optical sensitizer I-D and a  $\frac{1}{1000}$  mol methanol solution of optical sensitizer II-C in the amount or amounts shown on Table 5. The system was stirred for 30 minutes at 35° C. to stabilize the optical sensitization action and then applied to a film support followed by drying to provide a light-sensitive black and white element.

The film was cut into strips and they were subjected to yellow exposure through Fuji Filter No. 3 by means of a sensitometer at a color temperature of 2666° K. The thus exposed films were developed for 20 minutes at 20° C. in a D-76 (Eastman Kodak Co.) developer and then fixed to provide black and white negative images.

By measuring the densities of the negative images, the relative optical sensitizations were calculated. The results are shown in Table 5.

TABLE 5

| No.    | Amount of 1/1,000 mol methanol soln. of I-D (ml.) | Amount of 1/1,000 mol methanol soln. of II-D (ml.) | Relative color sensitization | $\mu$ |
|--------|---------------------------------------------------|----------------------------------------------------|------------------------------|-------|
| 1----- | 2                                                 | 0                                                  | 100                          | 654   |
| 2----- | 4                                                 | 0                                                  | 120                          | 543   |
| 3----- | 0                                                 | 2                                                  | 190                          | 686   |
| 4----- | 0                                                 | 4                                                  | 225                          | 686   |
| 5----- | 2                                                 | 2                                                  | 350                          | 698   |

<sup>1</sup>  $\mu$  = Maximum sensitization wave length.

What is claimed is:

1. A photographic silver halide emulsion containing at least one optical sensitizer represented by the following general Formula I and at least one optical sensitizer represented by the following general Formula II



(I-E)



and

8

Formula II



wherein  $R_1$ ,  $R_2$ ,  $R_3$ , and  $R_4$  each represents an alkyl group having 1 to 4 carbon atoms, a substituted alkyl group selected from the class consisting of hydroxyalkyl group, an acetoxyalkyl group, an alkylsulfate group, a carboxyalkyl group, a sulfoalkyl group, a carboxyalkoxalkyl group, a hydroxysulfoalkyl group, an alkoxy sulfonalkoxy alkyl group, a sulfoalkoxy alkoxy alkyl group or a hydroxy sulfoalkoxy alkyl group, an allyl group, an aralkyl group or a sulfo substituted aralkyl group, V represents a halogen atom;  $X^-$  represents an anion; and  $n$  is 1 or 2.

2. The photographic silver halide emulsion of claim 1 wherein said optical sensitizers of Formulas I and II are present in the emulsion in a ratio by weight in the range of from 9:1 to 1:9.

3. The photographic silver halide emulsion of claim 1 wherein the sensitizer of Formula I is a compound selected from the group consisting of



and the sensitizer of Formula II is a compound selected from the group consisting of

(II-A)



(II-B)



(II-C)

5



10

4. A photographic light-sensitive element comprising as a component the halide emulsion as claimed in claim 1.

## References Cited

15

## UNITED STATES PATENTS

|           |        |                |       |        |
|-----------|--------|----------------|-------|--------|
| 2,075,048 | 3/1937 | Nees           | ----- | 96—104 |
| 2,422,080 | 6/1947 | Collins et al. | ----- | 96—104 |
| 3,338,714 | 8/1967 | Ficken et al.  | ----- | 96—104 |

20

J. TRAVIS BROWN, Primary Examiner

U.S. Cl. X.R.

96—100